

1

3,840,462

**LUBRICANT COMPOSITIONS**Maximilian Geretschläger, Vienna, Austria, assignor to  
Mobil Oil CorporationNo Drawing. Filed June 9, 1972, Ser. No. 261,469  
Claims priority, application Austria, Apr. 7, 1972,  
3,036/72

Int. Cl. C10m 1/32, 3/26

U.S. Cl. 252—34.7

8 Claims

**ABSTRACT OF THE DISCLOSURE**

Lubricant compositions, particularly roll-oils, are provided, comprising in combination, a straight-chain fatty alcohol having from 1 to about 18 carbon atoms, a hydrocarbon fraction having a viscosity between about 28 and 100 SUS at 100° F., a fatty acid having from about 8 to about 22 carbon atoms, an ester of a fatty acid having from about 8 to about 22 carbon atoms and a fatty alcohol having from about 1 to about 18 carbon atoms, an organic amine, and a non-ionic emulsifier.

**CROSS-REFERENCE TO RELATED APPLICATIONS**

Austrian application 3,036/72, filed Apr. 7, 1972, priority for which is claimed.

**BACKGROUND OF THE INVENTION****(1) Field of the Invention**

This invention relates to lubricants which are suitable for the cold rolling of metals and their alloys. In one of its more specific aspects, the invention relates to cold rolling of aluminum and aluminum alloys and to roll-oil compositions adapted for such use. Still more particularly, in this aspect, the invention relates to lubricant compositions in the form of aluminum roll-oils which are not susceptible of causing white corrosion staining, thus reducing surface brightness of the metal, and other undesirable corrosion.

**(2) Description of the Prior Art**

Prior to the present invention, various lubricant formulations intended for use as roll-oil lubricants, particularly in the working of aluminum and its alloys, have been suggested. In employing such formulations, however, the rolling process has also resulted in causing white corrosion staining, thus also effecting reduction of surface brightness of the metal. Furthermore, in many instances, brown staining has also resulted, particularly at annealing temperatures. Other undesirable results encountered in the use of such formulations have included wettability of annealed foils due to oily conditions, corrosion on rolls and stands and the presence of comet tail marks.

**SUMMARY OF THE INVENTION**

In accordance with the present invention, it is now possible to provide improved lubricant compositions, particularly adapted for use as roll-oil lubricants in the working of metals such as aluminum and its alloys, in which undesirable white corrosion staining and reduction of metal surface brightness is avoided as well as achieving reduction of brown staining at annealing temperature, reduced wettability of annealed oils and the presence of undesirable comet tail marks. The improved lubricant compositions of the present invention, as more fully hereinafter described comprise:

(a) From about 5 to about 60%, by weight, of a straight-chain fatty alcohol having from 1 to about 18 carbon atoms,

2

- (b) from about 5 to about 70%, by weight, of a hydrocarbon fraction having a viscosity between about 28 and about 100 SUS at 100° F., and minor amounts of  
(c) a fatty acid having from about 8 to about 22 carbon atoms,  
(d) an ester of a fatty acid having from about 8 to about 22 carbon atoms and a fatty alcohol having from about 1 to about 18 carbon atoms,  
(e) an organic amine, and  
(f) from about 0.1 to about 50%, by weight, of a non-ionic emulsifier.

In preferred modifications (a) is present in an amount of from about 5 to about 35%, by weight; (b) is present in an amount from about 5 to about 48%, by weight; (c) is present in an amount from about 1 to about 10%, by weight; (d) is present in an amount from about 1 to about 20%, by weight; (e) is present in an amount from about 0.1 to about 5%, by weight; and (f) is present in an amount from about 0.1 to about 50%, by weight.

If so desired, various other improver additive components may be incorporated in the novel lubricant composition. Thus, for example, the lubricant composition may also contain, as an additional component, a fatty acid amine soap in an amount from about 0.5 to about 5%, by weight. Other additional components may include amine compounds of organic oxyacids in an amount from about 1 to about 5%, by weight, and also glycols in an amount from about 5 to about 30%, by weight. In a preferred modification component (b) may comprise a petroleum hydrocarbon fraction having an initial boiling point of from about 350° F. to about 525° F. and an end boiling point of from about 500° F. to about 620° F. Preferably, in the cold rolling of aluminum, the lubricant composition is employed in combination with water in lubricant concentrations of from about 1 to about 40%, by weight.

In the above-described lubricant compositions, and modifications thereof component (a) is present for the purpose of imparting film strength; component (b) is employed for imparting lubricity; component (c) is employed for imparting film strength and lubricity; component (d) is also employed for imparting lubricity; component (e) is employed as a corrosion inhibitor when employed in the form of a relatively high molecular weight amine, and as a preventor of white staining when employed in the form of a relatively low molecular weight amine; and component (f), as indicated, comprises the emulsifier. When employed as additional components, the fatty acid amine soap functions as a lubricating agent and a corrosion inhibitor; the amine compounds of organic oxyacids function as corrosion inhibitors; and the glycols function as solubilizers.

Exemplary of the straight-chain C<sub>1</sub>—C<sub>18</sub> fatty alcohol component (a) are lauryl, myristyl and palmityl alcohols or mixtures thereof. Exemplary of the hydrocarbon fraction of component (b) are narrow-cut high flash point kerosine fractions, having viscosities between about 28 and about 100 SUS at 100° F. Exemplary of the C<sub>8</sub>—C<sub>22</sub> fatty acid of component (c) are lauric, iso-stearic and oleic acids. Exemplary of the esters of fatty acids having from about 8 to about 22 carbon atoms and a fatty alcohol having from about 1 to about 18 carbon atoms of component (d) are methyloleate, butylmyristate, lauryl isostearate, and oleylcaprylate. Exemplary of the organic amine of component (e) are diethanolamine, amino-methylpropanol or mixtures of various alkylamines. Exemplary of the non-ionic emulsifier of component (f) are fatty acid alkylolamide and/or polyglycols or a mixture of polyglycols containing from 5-30 moles of ethyleneoxide derived from fatty alcohols, fatty acids, alkylphenols and/or polymerization products of ethyleneoxide and propyleneoxide. Exemplary of the fatty acid amine soaps are

triethanolamineoleate or the laurate of aminomethylpropanol. Exemplary of the amine compound of organic oxy-acids are the diethanolamine salt of the p-hydroxy-benzoic acid or the triethanolamine salt of the 3,4-dihydroxybenzoic acid-1.

In the above-described lubricant formulation of the present invention, it is found that if the fatty acid of component (c) contains less than about 8 carbon atoms, inferior load-carrying properties result. On the other hand, if the chain length of the acid is increased to above about 22 carbon atoms, formation of brown stains after annealing is intensified. These results are particularly apparent where the lubricant composition is employed in the form of an oil-in-water emulsion.

#### DESCRIPTION OF SPECIFIC EMBODIMENTS

The following examples and data will serve to illustrate the novel lubricant formulations of the present invention and their efficacy in the cold-rolling of metals.

The following oil-in-water roll-oil emulsions were prepared, as shown in the table and the degree of reduction in a single pass was determined on a foil rolling mill at a speed of 100 meters per minute. The initial thickness of the foil was 0.035 mm. The foil width was 420 mm. Lubricant A comprised an emulsion type fluid and lubricant B comprised a translucent type fluid. All measurements were recorded in percent by weight.

TABLE

| Components                                      | Lubricant A | Lubricant B |
|-------------------------------------------------|-------------|-------------|
| Lauryl alcohol                                  | 35.0        | 20.0        |
| Mineral oil (40 SUS at 100° F.)                 | 44.2        | 16.5        |
| Lauric acid                                     | 5.0         | 5.0         |
| Butyl stearate                                  | 10.0        | 10.0        |
| Diethanolamine                                  | 1.8         | 4.0         |
| Octylphenoxyethanol                             | 1.0         | 24.5        |
| Ethylene-propylene-oxide polymerization product |             | 5.0         |
| Hydroxy-benzoic acid-amine                      | 2.9         | 5.0         |
| Tetraethylene glycol                            |             | 10.0        |
| Silicone antifoamant                            | 0.1         |             |
| Total                                           | 100.0       | 100.0       |

Each of the above lubricant formulations were subjected to an experimental test on a finishing mill. This mill had a roll diameter of 50 mm. and a roll width of up to 140 mm. With loads up to 100 kp./cm.<sup>2</sup> reductions up to 85% were obtained. The surfaces of the individual foils and strips were excellent and free of appreciable evidence of white staining or other forms of corrosion.

As hereinbefore indicated, the improved lubricant compositions of the present invention may be employed as either emulsion type or translucent type roll-oil fluids. These lubricants are soluble in water in concentrations of from about 1 to about 40%, by weight. They are filterable through filter, earth-beds, paper, diffusion stones and similar materials, without deterioration or additive depletion to a pore width of the filter material of less than 0.3 microns. The rolling fluid containing a combination of selected additives exhibits a synergistic effect with respect to the straight-chain alcohol and the fatty acid ester and/or the fatty acid.

These lubricant fluids are biodegradable to a very high degree and are readily disposed. They exhibit good storage stability, particularly when employed in the emulsion form, and exhibit no rust formation on mills, rolls and on the material being rolled, with no formation of white or brown staining. Particularly with the translucent rolling fluid formulations, very bright surfaces can be obtained which are superior to those obtainable with common rolling oils, employing hydrocarbon fractions. The reduction ability to be effected is comparable with that of conventional rolling oils and in many instances exhibit superiority.

for rolling processes conducted at extremely high speeds. One of the most important features of the present rolling oils is their ability to withstand high rolling speeds up to 2,000 meters per minute and higher. By simple rearrangement of the formula components and adjustment of the specific rolling apparatus employed, rolling procedures are possible which exhibit high speed-low speed, high reduction-low reduction, relatively dull surfaces-bright surfaces.

In essence, the particular combination of lubricant components in the quantities hereinbefore described affords unusual properties not otherwise observed with lubricant compositions containing other components or similar components which are present in amounts falling outside the aforementioned critical range.

It will be understood that although the present invention has been described with preferred embodiments, various modifications and adaptations thereof may be resorted to without departing from the spirit and scope of the invention as those skilled in the art will readily understand.

I claim:

1. A lubricant composition comprising:
  - (a) from about 5 to about 60%, by weight, of a straight-chain fatty alcohol having from 1 to about 18 carbon atoms;
  - (b) from about 5 to about 70%, by weight, of a hydrocarbon fraction having a viscosity between about 28 and about 100 SUS at 100° F.;
  - (c) from about 1 to about 20%, by weight, of a fatty acid having from about 8 to about 22 carbon atoms;
  - (d) from about 1 to about 30%, by weight, of an ester of a fatty acid having from about 8 to about 22 carbon atoms and a fatty alcohol having from about 1 to about 18 carbon atoms;
  - (e) from about 0.1 to about 10%, by weight, of an organic amine; and
  - (f) from about 0.1 to about 50%, by weight, of a non-ionic emulsifier.

40 2. A lubricant composition as defined in Claim 1 wherein said lubricant is employed in combination with water in lubricant concentrations of from about 1 to about 40%, by weight.

45 3. A lubricant composition as defined in Claim 1 wherein (a) is present in an amount of from about 5 to about 35%, by weight; (b) is present in an amount from about 5 to about 48%, by weight; (c) is present in an amount from about 1 to about 10%, by weight; (d) is present in an amount from about 1 to about 20%, by weight; (e) is present in an amount from about 0.1 to about 5%, by weight; and (f) is present in an amount from about 0.1 to about 10%, by weight.

50 4. A lubricant composition as defined in Claim 1 wherein (b) comprises a petroleum hydrocarbon fraction having an initial boiling point of from about 350° F. to about 525° F. and an end boiling point of from about 500° F. to about 620° F.

55 5. A lubricant composition as defined in Claim 1 wherein (a) comprises from about 20 to about 35%, by weight, lauryl alcohol; (b) comprises from about 16.5 to about 44.2%, by weight, of a mineral oil having a viscosity of 40 SUS at 100° F.; (c) comprises about 5%, by weight, lauric acid; (d) comprises about 10%, by weight, butyl stearate; (e) comprises from about 1.8 to 4%, by weight, diethanolamine; and (f) comprises from about 1 to about 24.5%, by weight, octylphenoxyethanol.

60 6. In the rolling of metals and their alloys, the method of lubricating which comprises applying to the metal or alloy, at a point prior to the work rolls, a lubricant composition as defined in Claim 1.

70 7. In the rolling of metals and their alloys, the method of lubricating which comprises applying to the metal or alloy, at a point prior to the work rolls, a lubricant composition as defined in Claim 2.

8. In the rolling of metals and their alloys, the method of lubricating which comprises applying to the metal or

alloy, at a point prior to the work rolls, a lubricant composition as defined in Claim 3.

|           |         |                     |            |
|-----------|---------|---------------------|------------|
| 2,780,598 | 2/1957  | Cafcas -----        | 252—34.7 X |
| 3,507,791 | 4/1970  | Teeter et al. ----- | 252—34.7   |
| 3,390,084 | 6/1968  | Lake -----          | 252—34.7   |
| 3,392,116 | 7/1968  | Hornus -----        | 252—34.7 X |
| 3,630,898 | 12/1971 | Teeter et al. ----- | 252—34.7   |

## References Cited

## UNITED STATES PATENTS

|           |         |                     |            |
|-----------|---------|---------------------|------------|
| 1,990,365 | 2/1935  | Beale -----         | 252—34.7 X |
| 2,025,435 | 12/1935 | Bouhuys -----       | 252—34.7 X |
| 2,625,509 | 1/1953  | Laug -----          | 252—34.7   |
| 2,668,146 | 2/1954  | Cafcas et al. ----- | 252—34.7 X |

5

HELEN M. S. SNEED, Primary Examiner

U.S. Cl. X.R.

10 252—51.5 R, 56 R